

Aug. 11, 1931.

R. L. WHITE

1,818,876

PAVING MATERIAL AND PROCESS OF MANUFACTURING THE SAME

Filed Nov. 5, 1929



Patented Aug. 11, 1931

1,818,876

# UNITED STATES PATENT OFFICE

RYALL L. WHITE, OF SAN ANTONIO, TEXAS

## PAVING MATERIAL AND PROCESS OF MANUFACTURING THE SAME

Application filed November 5, 1929. Serial No. 404,970.

This invention relates to improvements in paving materials, and to a novel method or process for manufacturing such materials.

Asphaltic or bituminous paving materials heretofore used have generally been mixed and applied directly at the roadway to be surfaced, or have been premixed at the plant and maintained in heated condition until the time of laying. Some effort has also been made to mix such materials at the mines or the like, and to incorporate in the materials, substances to keep the adhesive inactive until the material was actually spread on the roadway to be surfaced. This latter effort has disadvantages, due to the expense involved.

The primary object of the present invention is to eliminate the disadvantages inherent in the prior paving materials, and present in the methods employed; and in accordance with my invention, the materials are mixed at the mine, and are so balanced that the mixture may be shipped to distant points and remain inert until such time as it is spread. When the mixture is spread, the water which maintains the same inert, while in bulk, rapidly evaporates, and the mixture hardens and properly sets, thus securing a more uniform and less expensive job than was formerly possible by the mixing of the material in situ by workmen of limited experience.

Another object of this invention is to furnish a method in which a crude oil having a comparatively high Baumé gravity and low asphaltic content, is first added to pulverized rock asphalt at the quarry for the purpose of securing a preliminary fluxing and softening effect on the rock asphalt. Then a crude oil having a comparatively low Baumé gravity and high asphaltic content is added to the mixture, for the purpose of furnishing additional bitumen to give the necessary binding or adhesion, and finally a proper amount of water is added to render the adhesive qualities of the asphalt temporarily inactive, so that the mixture, while shipped or stored in bulk, will have the desired plasticity. When, however, such mixture is spread, the aqueous

moisture therein will evaporate, and permit the binding substances to again become active, whereby the mixture rapidly hardens and properly sets.

From the above it will be understood that my improved paving material in bulk condition, will consist of pulverized rock asphalt or the like, a fluxing oil having a comparatively high Baumé gravity, and low asphaltic content; a fluxing oil having a comparatively low Baumé gravity and a high asphaltic content; and sufficient water to render the adhesive qualities of the asphalt temporarily inactive. When such material is spread, and after hardening and setting, it will be of about the same composition, minus all or substantially all of its water content.

Various apparatus may be employed in the manufacture of my paving material, and one form of suitable apparatus is illustrated in the accompanying drawing, which shows a diagrammatic view of such an apparatus.

Referring to the method of manufacture in detail, in connection with this drawing, the rock asphalt or the like, when received from the quarry, is discharged from the dump car A into a 42 inch crusher B, which may be of the Superior McCully gyratory type. The discharge opening at the bottom of this crusher is three and one-half inches in area, and the rock asphalt, after passing through the crusher, is discharged into a pan conveyor C, and elevated to the top of a steel bin D, where it is discharged on to an apron conveyor E and distributed the full length of the bin.

As the pulverized rock asphalt or the like, used in my paving material, varies from three-eighths to one-half inch in size, the material is conveyed from the bottom of the bin by an apron conveyor F, and discharged into a suitable pulverizer G, which reduces the same to proper size. After the material is pulverized, it passes into a bucket conveyor H which elevates the same approximately sixty feet. From this elevation, it is either discharged into a railroad car I, in case just regular run pulverized rock asphalt is required, or if it is to be employed in pre-

paring my improved paving material, it is discharged into a chute J which leads to the bottom of another small bucket elevator K, used in connection with the mixing plant. After passing into the bucket elevator of the mixing plant, it is elevated to a height of approximately thirty feet, and is discharged into a hopper L, where it is measured off in batches of say 1500 pounds per batch. From this hopper, the pulverized rock asphalt or the like passes into a suitable mill M, of the pug or drum type. While the mill is operating on the batch, approximately three gallons of the first flux oil is added, and thoroughly mixed with the pulverized material. This flux oil is preferably a crude oil having a comparatively high Baumé gravity and low asphaltic content for the purpose of securing a preliminary fluxing and softening effect. Such oil may have the characteristics of the Luling product, which are as follows:

|                      |              |
|----------------------|--------------|
| Gravity              | 27           |
| Flash                | 110° F.      |
| 25 Sulphur           | 68/100 of 1% |
| B. S. & W.           | 1/2 of 1%    |
| Cold test            | 10% F.       |
| Viscosity            | 1.81 @ 70%   |
| Percent              |              |
| 30 Naphtha           | 7.3          |
| Kerosene             | 5.0          |
| Gas oil              | 27.7         |
| Crude lube           | 35.7         |
| 35 Asphalt           | 19.7         |
| Loss by distillation | 4.6          |
|                      | 100.0        |

This first flux oil may be fed to the mixing mill from a measuring tank N, through a valved pipe line O.

After this flux oil has been thoroughly mixed with the pulverized material, approximately three gallons of a second flux oil from a measuring tank P may be fed into the material in the mill M, through a valved pipe line Q. This second flux oil preferably should have a comparatively low Baumé gravity and a high asphaltic content for the purpose of furnishing additional bitumen to give the necessary binding or adhesion to the finished paving material. I have found Hondo crude admirably adapted for this purpose. It tests as follows:

|                                              |               |
|----------------------------------------------|---------------|
| 55 Gravity A. P. I.                          | 16            |
| Flash point                                  | 187° F.       |
| Asphalt content                              | 63%           |
| Total bitumen (soluble in carbon disulphide) | 99.5%         |
| 60 Organic matter insoluble                  | 0.00          |
| Water                                        | 0.1%          |
| Sediment                                     | 0.1% B. S. W. |

Instead of using Hondo, I may use any flux oil having similar characteristics. For

example, I have also used in the mixture in substitution for the Hondo crude, an oil testing as follows:

|                           |          |
|---------------------------|----------|
| Sp. gravity @ 60° F.      | .9541    |
| Gravity, A. P. I.         | 16.8     |
| Flash, C. O. C. °F.       | 195° F.  |
| Viscosity, Furol @ 77° F. | 363 sec. |
| Bottom sediment           | 0.1%     |
| Water                     | 0.0%     |

75

After the flux oils have been thoroughly mixed with the pulverized material, approximately six gallons of water is added to the batch and admixed into the mixture. The mixture remains in the mill M for a period of approximately two minutes, and is then discharged into a railroad car R or the like, for shipment to the point of utilization.

As before stated, the water will render the adhesive qualities of the asphalt inactive until such time as the water evaporates. Obviously, if the finished material is in bulk, there will be less tendency for the aqueous moisture to depart than if the material is spread out in a relatively thin layer.

While I have disclosed my invention in such manner that the same may be readily understood by those skilled in the art, I am aware that changes may be made in the specific materials employed, and in the details of the method, without departing from the spirit of the invention, as expressed in the appended claims.

What I claim and desire to secure by Letters Patent is:

1. Paving material comprising pulverized rock asphalt, sufficient flux oil having comparatively high Baumé gravity and low asphaltic content, but containing appreciable quantities of asphalt, to secure a preliminary fluxing and softening effect on the rock asphalt, a sufficient quantity of a second asphaltic flux oil sufficiently fluid at ordinary temperatures so that it can be thoroughly mixed cold with the rock asphalt, said second flux oil having a comparatively low Baumé gravity and high asphaltic content for the purpose of furnishing additional bitumen to give the necessary binding qualities to the material, and a sufficient quantity of water to render the adhesive qualities of the asphalt temporarily inactive.

2. The paving material as in claim 1, wherein the proportions of ingredients are approximately as follows, 1500 pounds of rock asphalt, 3 gallons of flux oil of comparatively high Baumé gravity and low asphaltic content, 3 gallons of asphaltic oil of comparatively low Baumé gravity and high asphaltic content, and 6 gallons of water.

RYALL L. WHITE.

130